

# UNITED STATES PATENT OFFICE.

MAURICE PONTIO, OF PARIS, FRANCE.

## MOLDED OBJECT IN IMITATION OF PORCELAIN.

1,293,191.

Specification of Letters Patent.

Patented Feb. 4, 1919.

No Drawing.

Application filed June 1, 1917. Serial No. 172,335.

To all whom it may concern:

Be it known that I, MAURICE PONTIO, citizen of the Republic of France, residing at 7 Rue Legraverend, Paris, in the Republic of France, have invented new and useful Improvements in Molded Objects in Imitation of Porcelain, of which the following is a specification.

The object of the present invention is the manufacture of heads and bodies for dolls and in general the production of all objects capable of being molded, especially busts, statuettes, bases, dress forms, artificial limbs, photographic trays or dishes for various purposes and divers parts for all kinds of apparatus, such manufacture being carried out by the following process.

The material used for producing these objects consists essentially of a mixture of mineral powders, such as talc, kaolin, plaster of Paris, Spanish white, or Meudon white, etc., made up by the use of an aqueous solution of gelatin or gelose mixed with casein, such mixture being used alone or together with gum arabic or any other adhesive mucilaginous substance.

In this way, there is formed a paste which is applied in successive layers in a mold in order to obtain dolls' heads and bodies, and these are afterward rendered insoluble by placing them in a bath of formic aldehyde or any other product which will render gelatin insoluble. After drying, the material is decorated and varnished as may be required.

Hardening is produced by the drying of the material, in which the gelatin has been rendered insoluble by the action of the formol.

As the process of rendering material insoluble by formol is a very slow one, there is no disadvantage in using the action of the latter before the molding, if desired, for the paste will remain liquid for a certain time. In this latter case the paste containing the formol already added, is applied in successive layers in the mold as above mentioned, and after drying it is decorated and varnished as may be required.

It will thus be seen that the formol treatment can be carried out either before or 50 after the molding.

The following method of operating is preferable:

The operation is commenced by dissolving casein in a water bath in a certain quantity 55 of boiling water (with a minimum of 10 grams of casein per 100 grams water) this being rendered alkaline by adding a few drops of ammonia or caustic soda solution. The casein can be considered as sufficiently 60 dissolved when no grains are seen upon the bottom of the vessel.

To the above solution there is added sheet gelatin (with a minimum of 10 grams of gelatin per 100 grams water), then gum 65 arabic ( $\frac{1}{4}$  of the weight of the gelatin) which has been previously dissolved in hot water and filtered through cloth, and lastly the mineral powders in variable quantity and number according to the appearance and 70 size of the object which it may be desired to obtain, as well as the required amount of coloring matter to obtain the desired color for the paste. This mixture is stirred constantly until it becomes quite homogeneous 75 and is then allowed to cool, but this under a constant stirring. While still in the liquid state, the above paste is used to prepare a hollow object by applying it in successive layers inside a mold, and it is allowed to 80 solidify until completely cold. The molded object is now removed from the mold and placed for several hours in a 15 per cent. formol solution, then it is dried in an oven whose temperature is gradually varied from 85 25 to 80 degrees centigrade. Lastly, it is polished and decorated according to the case.

Objects obtained by this process are very strong, and the expense is a minimum. 90

Having now described my invention what I claim as new and desire to secure by Letters Patent is:

1. A molded object in imitation of porcelain containing an impalpable powder, a coloring substance, a solution of alkaline case-

inate, an aqueous solution of gelatin, a gum and formol, substantially as described and for the purpose set forth.

2. A molded object in imitation of porcelain containing an impalpable powder, a solution of alkaline caseinate, an aqueous solution of gelatin, a gum, and formol, substantially as described.

In testimony whereof I have signed my name to this specification in the presence of 10 two subscribing witnesses.

MAURICE PONTIO.

Witnesses:

LOUIS MOSES,  
CHAS. P. PRESSLY.